

Aug. 6, 1935.

E. AYRES ET AL

2,010,387

TREATING LUBRICATING OILS

Filed Aug. 11, 1932



Inventors  
Eugene Ayres,  
Herschel G. Smith,

By *G. M. Daugherty*  
Attorney

## UNITED STATES PATENT OFFICE

2,010,387

## TREATING LUBRICATING OILS

Eugene Ayres and Herschel G. Smith, Swarthmore, Pa., assignors to Gulf Refining Company, Pittsburgh, Pa., a corporation of Texas

Application August 11, 1932, Serial No. 628,446

12 Claims. (Cl. 196—78)

This invention relates to treating lubricating oils; and it comprises a process wherein a lubricating oil stock is mixed with a small percentage of aluminum chloride and with a halogenated hydrocarbon, such as an alkyl, aralkyl, alkylene or aryl halide, usually containing not more than one halogen atom attached to any one carbon atom, the mixture is heated at moderate temperatures and the resulting sour oil is sweetened and purified; all as more fully hereinafter set forth and as claimed.

Within the past few years there has arisen an important demand for lubricating oils of diverse but specific properties. The usual procedure employed to obtain oils with specific properties has been to derive such oils from an appropriate crude petroleum, because each crude is capable of yielding oils of certain characteristic properties. It has not always been possible, however, to obtain certain extreme combinations of properties by the ordinary refining methods, and it has not always been practicable to depend upon the availability of a sufficient variety of crudes to satisfy market demands. Various methods have been proposed for the modification of the properties of lubricating oils to simulate in certain respects the properties of lubricating oils from other types of crude, but all such methods have been of limited usefulness. Some of the methods, such as extraction with liquid sulfur dioxide, are limited in the degree of change of properties, and other methods, such as hydrogenation, are limited in the direction in which the change is effected. Hydrogenation, for example, is incapable of increasing the viscosity of the oil and is also incapable of producing a lower viscosity index. For many applications a high viscosity index is desired, but in some applications, such as the preparation of certain greases, very low viscosity indices are required. This invention offers a flexible method by which any property of a lubricating oil may be changed in either direction at will by selection of suitable conditions.

In a copending application, Serial No. 598,096, filed March 10, 1932, we have described a method of improving various hydrocarbon products by treating a mixture of inferior technical stocks, or one of said stocks, at low temperatures with a chlorine containing gas and, either simultaneously or subsequently, with aluminum chloride. The present invention represents, in some respects, an improvement upon or an extension of the process of this prior application.

We have found that, by treating various lubri-

cating oils with halogenated hydrocarbons in the presence of aluminum chloride and at moderate temperatures, a remarkable and specific alteration of their properties is effected. The characteristics of such stocks are changed in various ways, depending to some extent upon the nature of the chlorinated hydrocarbon used and upon the conditions of treatment. In general, treatment with halogenated hydrocarbons having not more than a single halogen atom attached to any one carbon atom increases the A. P. I. gravity, lowers the carbon residue and raises the viscosity as well as the viscosity index. By this method, for example, coastal lubricating oils having low gravity, viscosity and viscosity index can be so far improved that their properties approach those of the best grade paraffin type, mid-continent oils. But by selection of the particular hydrocarbon halide used in the process, it is possible to change the properties of an oil almost at will.

In our process the oil to be treated is mixed with a substantial amount, say 5 to 100 per cent by weight, of chlorinated hydrocarbon, such as an alkyl, alkylene, or aryl mono- or poly-halide, a small amount of aluminum chloride (usually from 1 to 10 per cent) is added and the resulting mixture is heated under agitating conditions to temperatures ranging from about 150° to 300° F. A closed container may be used, if desired. The time of treatment may range from a few minutes up to several hours, depending to some extent upon the temperature employed, the amount of aluminum chloride used and the efficiency of agitation. The sludge formed in the process is separated and the remaining sour oil is sweetened and purified, usually by heating with fuller's earth and lime, followed by filtration. The halogenated hydrocarbon disappears in the process, the halogen content being eliminated in the form of the corresponding hydrogen halide.

The alteration in the properties of the oil may possibly be explained on the theory that a synthesis takes place, the hydrocarbon residue from the halogenated compound uniting with certain hydrocarbons found in the oil. While this is a possible explanation it would be extremely difficult to substantiate such a theory in practice.

To illustrate our process in more detail several illustrative examples will be given which represent practical embodiments of the invention.

*Example 1.*—One hundred volumes of a coastal lubricating distillate were agitated in a closed container with 10 per cent by weight of aluminum chloride for two hours at a temperature of 175°

5

10

15

20

25

30

35

40

45

50

55

F. and under a pressure of 100 pounds of ethyl chloride. After treatment, the sludge was permitted to settle and the sour oil was decanted. The latter was then steamed at 450° F. with 0.5 pound of fine Florida clay per gallon of oil and 0.6 pound of lime per acid number per barrel. After steaming the oil was filtered. The yield of finished oil was found to be 70 volumes, showing the following comparative tests:

10

|                             | Charging stock | Product |
|-----------------------------|----------------|---------|
| Gravity: ° A. P. I.         | 20.7           | 23.7    |
| Viscosity, S. U. V. 210° F. | 75             | 76      |
| Viscosity index             | 17             | 54      |
| Flash, O. C.: ° F.          | 415            | 455     |
| Fire, O. C.: ° F.           | 495            | 525     |
| Color, N. P. A.             | 5.5            | 2.0     |
| Carbon residue: Percent     | 0.27           | 0.07    |

20

This example illustrates an improvement of the oil by increase in gravity and viscosity index, the viscosity at 210° F. remaining about the same. The carbon residue is reduced.

25

*Example 2.*—One hundred volumes of the same coastal lubricating distillate used in Example 1, were stirred with 10 per cent of aluminum chloride and with 30 volumes of amyl chloride for 2 hours at a temperature of 175° F. The oil was finished in the same manner as that employed in Example 1. Seventy volumes of finished oil were obtained showing the following comparative tests:

35

|                             | Charging stock | Product |
|-----------------------------|----------------|---------|
| Gravity: ° A. P. I.         | 20.7           | 24.2    |
| Viscosity, S. U. V. 210° F. | 75             | 101     |
| Viscosity index             | 17             | 55      |
| Flash, O. C.: ° F.          | 415            | 460     |
| Fire, O. C.: ° F.           | 495            | 530     |
| Color, N. P. A.             | 5.5            | 2.75    |
| Carbon residue: Percent     | 0.27           | 0.44    |

In this example the gravity, viscosity and viscosity index of the lubricating stock are raised by treatment with amyl chloride and aluminum chloride.

*Example 3.*—One hundred volumes of the same coastal lubricating distillate as that used in Example 1 were agitated with 10 per cent of aluminum chloride and with 30 volumes of amylene dichloride for 2 hours at 175° F. The oil was finished in the same manner as in Example 1. Ninety-eight volumes of finished oil were obtained showing the following comparative tests:

55

|                             | Charging stock | Product |
|-----------------------------|----------------|---------|
| Gravity: ° A. P. I.         | 20.7           | 19.9    |
| Viscosity, S. U. V. 210° F. | 75             | 141     |
| Viscosity index             | 17             | 20      |
| Flash, O. C.: ° F.          | 415            | 445     |
| Fire, O. C.: ° F.           | 495            | 525     |
| Color, N. P. A.             | 5.5            | 7.0 dl. |
| Carbon residue: Percent     | 0.27           | 3.27    |

65

This example illustrates a method of producing an extraordinary increase of viscosity with some increase in viscosity index, these changes being coupled with an increase in carbon residue.

*Example 4.*—One hundred volumes of mid-continent bright stock were stirred with 10 per cent of aluminum chloride and 50 volumes of amyl chloride for 2 hours at a temperature of 220° F. The oil was finished in the same manner as above. Eighty volumes of the finished

oil were obtained showing the following comparative tests:

|                             | Charging stock | Product |
|-----------------------------|----------------|---------|
| Gravity: ° A. P. I.         | 23.0           | 27.9    |
| Viscosity, S. U. V. 210° F. | 151            | 94      |
| Viscosity index             | 73             | 98      |
| Flash, O. C.: ° F.          | 545            | 500     |
| Fire, O. C.: ° F.           | 630            | 585     |
| Pour: ° F.                  | +15            | +20     |
| Color, N. P. A.             | 7.5            | 3.75    |
| Carbon residue: Percent     | 1.75           | 0.23    |

In this example the gravity of the oil is raised markedly, the viscosity index is increased and the carbon residue reduced.

*Example 5.*—One hundred volumes of a low viscosity Pennsylvania type distillate were stirred with 5 per cent of aluminum chloride and with 50 volumes of amylene dichloride for 4 hours at a temperature of 175° F. The oil was finished as in Example 1. One hundred twelve volumes of finished oil were obtained showing the following comparative tests:

|                             | Charging stock | Product |
|-----------------------------|----------------|---------|
| Gravity: ° A. P. I.         | 28.5           | 28.4    |
| Viscosity, S. U. V. 210° F. | 58             | 73      |
| Viscosity index             | 95             | 79      |
| Flash, O. C.: ° F.          | 440            | 465     |
| Fire, O. C.: ° F.           | 505            | 530     |
| Color, N. P. A.             | 2.25           | 7.5     |

This example illustrates the possibility of increasing the viscosity of an oil without substantial lowering of the A. P. I. gravity.

*Example 6.*—One hundred volumes of mid-continent bright stock were agitated with 2 per cent of aluminum chloride and 15 volumes of benzyl chloride for 1 hour at a temperature of 150° F. The oil was finished as above. Fifty-eight volumes of oil were obtained showing the following comparative tests:

|                             | Charging stock | Product |
|-----------------------------|----------------|---------|
| Gravity: ° A. P. I.         | 22.8           | 26.3    |
| Viscosity, S. U. V. 210° F. | 156            | 122     |
| Viscosity index             | 85             | 90      |
| Flash, O. C.: ° F.          | 545            | 545     |
| Fire, O. C.: ° F.           | 605            | 610     |
| Pour: ° F.                  | +15            | +20     |
| Color, N. P. A.             | 4.75           | 3.25    |
| Carbon residue: Percent     | 1.42           | 0.34    |

This table shows that a marked rise in A. P. I. gravity is produced by treatment with an aralkyl chloride. The carbon residue is lowered and the viscosity index is raised slightly.

*Example 7.*—One hundred volumes of mid-continent bright stock, the same as that used in Example 6, were stirred with 6 per cent of aluminum chloride and with 25 volumes of ortho dichlorobenzene for 2 hours at a temperature of 110° F. The oil was finished as in Example 1. Seventy-six volumes of oil were obtained showing the following comparative tests:

|                             | Charging stock | Product |
|-----------------------------|----------------|---------|
| Gravity: ° A. P. I.         | 22.8           | 25.4    |
| Viscosity, S. U. V. 210° F. | 156            | 152     |
| Viscosity index             | 85             | 88      |
| Flash, O. C.: ° F.          | 545            | 545     |
| Fire, O. C.: ° F.           | 605            | 625     |
| Pour: ° F.                  | +15            | +20     |
| Color, N. P. A.             | 4.75           | 4.25    |
| Carbon residue: Percent     | 1.42           | 0.66    |

In this example the fire test was improved and the carbon residue lowered, with slight increases in gravity and viscosity index.

Example 8.—One hundred volumes of reduced Oklahoma crude were agitated in a closed container with 10 per cent of aluminum chloride and 10 per cent of chloroform for 2 hours at a temperature of 150° F. The sour oil was decanted from the aluminum chloride sludge and agitated with 5 per cent sulfuric acid for a time sufficient to decompose the suspended particles of aluminum chloride sludge. After settling out the dilute acid wash, the oil was contacted with fine clay and finally filtered through coarse burned clay. Ninety-nine volumes of oil were obtained showing the following comparative tests:

|                             | Charging stock | Product  |
|-----------------------------|----------------|----------|
| Gravity: A. P. I.           | 19.8           | 10.4     |
| Viscosity, S. U. V. 210° F. | 138            | 159      |
| Viscosity index             | 74             | bel. -20 |

This example illustrates the possibility of markedly lowering the viscosity index and the A. P. I. gravity by the use of halogenated hydrocarbons having more than one halogen atom connected to a single carbon atom.

Example 9.—One hundred volumes of the same stock as that used in Example 8 were stirred with 10 per cent of aluminum chloride and 20 volumes of chlorinated naphthalene for 2 hours at 175° F. The oil was finished as in Example 1. Fifty volumes of oil were obtained showing the following comparative tests:

|                             | Charging stock | Product |
|-----------------------------|----------------|---------|
| Gravity: A. P. I.           | 19.8           | 25.0    |
| Viscosity, S. U. V. 210° F. | 138            | 103     |
| Viscosity index             | 74             | 93      |
| Flash, O. C.:° F.           | 460            | 510     |
| Fire, O. C.:° F.            | 560            | 580     |

The above data illustrate the raising of the viscosity index and the A. P. I. gravity by treatment with halogenated aryl compounds.

While the above examples illustrate what we consider the best embodiments of our invention, various changes can be made without departing from the scope of our invention. The above examples have been chosen to illustrate various types or classes of halogenated hydrocarbons which are applicable in our process. While in most cases only a single example of a group of compounds is given, our experiments indicate that substantially all members of the groups illustrated are equally operative. Typical members of alkyl, alkylene, aralkyl, and aryl halides are given to illustrate the action of these groups as a whole. Among other halogenated hydrocarbons, suitable for raising the A. P. I. gravity and viscosity index of lubricating oils, having low values of these constants, there may be mentioned the monochlorides of methane, propane, butanes, hexanes, etc., dichlorides of the ethylene dichloride series, and the products from the moderate chlorination of fractions of petroleum, including wax. It will be noted that all of these compounds have at least one halogen atom connected to a carbon atom, but not more than one connected to any one carbon atom, this forming the common characteristic which makes them operative in this particular relation. While

chlorine is the only halogen illustrated in the examples, bromine substituted hydrocarbons are also applicable. In commercial operation, however, the cost of these compounds is usually prohibitive.

On the other hand, if it is desired to lower the A. P. I. gravity and the viscosity index, use may be made of halogenated hydrocarbons having more than one halogen atom connected to a single carbon atom. As additional examples of such compounds there may be cited dichlorides of the ethylenedichloride series, trichlorethylene with its homologues, and the products of severe chlorination of fractions of petroleum. These examples illustrate other specific effects produced by typical halogenated hydrocarbons.

As will be noted by studying the above examples, the results produced are not conditioned solely by the type of chlorinated hydrocarbon used, but also depend to some extent upon the temperature, pressure and the time employed during treatment, as well as upon the amounts of aluminum chloride and chlorinated hydrocarbon used. With the aid of these examples as a guide it is a rather simple matter to alter the characteristics of any given lubricating oil to meet specifications of rather diverse character.

Various methods can be used for finishing or purifying the sour oil resulting from treatment with aluminum chloride and halogenated hydrocarbon. The above examples illustrate at least two suitable methods. A third method which may be mentioned is a simple heating of the sour oil to temperatures at which the traces of suspended aluminum chloride sludge will completely react with the oil. This temperature is usually between 450° and 550° F. After the sludge is spent, the oil can be clarified by filtration.

The time of treatment required varies to some extent with the temperatures and pressures employed. At atmospheric pressures usually from 1 to 2 hours are required for treatment, while at 100 pounds pressure and temperatures approaching 300° F., from 10 to 15 minutes is usually sufficient. In any case heating should be continued until reaction is complete.

In certain cases it has been found advantageous to fractionate the oil after treatment to separate out certain undesirable constituents. When treating lubricating oils containing unsaturated or naphthenic lubricating fractions by our process, we sometimes secure lubricating oils that are mixtures of oils of improved quality with some fractions of inferior quality. A fraction, usually a high boiling fraction, is sometimes found in the treated oil having such characteristics as a low gravity, low viscosity index and a comparatively high carbon residue. Where such characteristics are not desired in the finished oil, a considerable improvement can usually be obtained by distilling such a treated oil, any inferior fractions being discarded. In some cases the residuum obtained from such fractionation is found to have a quality superior to that of the distillate. In this case fractionation is of great advantage in producing a heavier oil of better grade.

Our invention may be illustrated with greater clarity by reference to the accompanying drawing, which shows, in the form of a flow sheet, a typical process within the purview of our invention, wherein a lubricating oil stock is mixed with a halogenated hydrocarbon and the mixture is treated by a series of successive operations, with

the ultimate production of a finished lubricating oil of improved properties. The several successive operations are indicated on the flow sheet by appropriate legends.

5 Referring to the flow sheet, a lubricating oil stock is shown introduced into an agitator together with a halogenated hydrocarbon. Optionally, the halogenated hydrocarbon may be added under pressure. The halogenated hydrocarbon 10 is of that type of compound in which at least one halogen atom is connected to a carbon atom, but not more than one halogen atom is connected to any one carbon atom.

15 Aluminum chloride is introduced into the agitator and the mixture agitated until the reaction is completed, after which the mixture is removed from the agitator to a sludge separator where the sludge is permitted to settle and is drawn off. As shown in the flow sheet, the remaining sour 20 oil may be finished by one of several alternative procedures.

If an acid finishing step is desirable, the sour oil from the sludge separator is introduced into an agitator and there agitated with weak sulfuric acid for a time sufficient to decompose the suspended particles of aluminum chloride sludge, after which the mixture is settled in a sludge separator, the acid sludge drawn off and the remaining oil passed first through a fine clay and 30 finally through a coarse clay filter. After filtration, the oil may be recovered as a finished lubricating oil. Optionally, however, it is desirable in some instances to fractionate the oil at this stage.

35 If, on the other hand, it is desired to finish sour oil by a treatment different from that just described, such sour oil may be introduced into a fire and steam still and heated to a temperature at which the traces of suspended aluminum chloride sludge completely react with the oil. At this stage, if desired, instead of a simple heating of the oil, the latter may be steamed at around 450° F. with clay and lime. In either event, the halogenated hydrocarbon disappears at this stage, the 40 halogen content being driven off from the still and recovered in the form of the corresponding hydrogen halide. After either the simple heating or the treatment with clay and lime, the sweetened oil is filtered and recovered at this 45 stage as a finished lubricating oil. In some instances the finished oil is fractionated in the same manner as previously described.

The proportion of aluminum chloride used in our process can be varied widely. Usually from 55 1 to 10 per cent by weight of the lubricating oil stock is found to be sufficient. Use of larger proportions is usually attended with larger losses. A balance may usually be struck between the improvement desired in the oil, such as increase in 60 viscosity, and the loss to sludge.

The proportions of halogenated hydrocarbon used in the process can likewise be varied widely. Depending to some extent upon the nature of the halogenated hydrocarbon involved and the 65 change in characteristics desired, proportions ranging from 5 to 100 per cent by weight, based on the lubricating stock, can be employed advantageously. When the higher proportions of a halogenated hydrocarbon are employed it is frequently possible to obtain a yield of over 100 per 70 cent, based on the lubricating stock. Such a yield is shown in Example 5, for instance. It will be noted from the above examples that amyl chloride and amylene dichloride give excellent results 75 in increasing viscosity and viscosity index, as well

as in producing high yields. We therefore consider these chlorides to be the most advantageous of the chlorinated hydrocarbons tested.

The simple admixture of light chlorinated hydrocarbons, such as ethyl chloride and amylene dichloride, for example, with lubricating oils produces a substantial reduction in viscosity. In contrast to this our process usually results in a lubricating oil of increased viscosity, even when such compounds are employed in quantities up to 50 per 10 cent or more by weight. As mentioned, the chlorine is eliminated from the reaction mixture as hydrogen chloride. There is no yield of a light hydrocarbon corresponding to the chlorinated hydrocarbon employed. These facts indicate that 15 our reaction is a synthesis, the residues of the halogenated hydrocarbons being combined with other residues during the reaction.

In many cases the operating procedure may be varied, within the scope of the following claims, 20 to suit the particular material which is being treated or the particular product it is desired to produce. Some of these variations have been indicated above while others will be evident to those skilled in the art.

What we claim is:

1. In the treatment of lubricating oil, the process which comprises mixing a lubricating stock with a small percentage of aluminum chloride and with a low boiling halogenated hydrocarbon having not more than a single halogen atom attached to any one carbon atom, subjecting the mixture to a treatment substantially equivalent to that obtained by heating for from 1 to 2 hours at atmospheric pressure and at temperatures ranging from about 150° to 300° F., decanting the resulting sour oil, decomposing traces of aluminum chloride sludge that remain in the sour oil by a method selected from a group consisting of, first, steaming the sour oil with a small amount of clay and with about 0.6 pound of lime per acid number per barrel, second, agitating with dilute sulfuric acid for a time sufficient to decompose suspended particles of sludge, separating the acid 30 and contacting with clay, third, heating said sour oil to temperatures at which the traces of suspended sludge will completely react with the oil; then filtering the decomposed particles of sludge from the oil and recovering a finished oil of increased viscosity index, low color N. P. A. and low 35 carbon residue.

2. In the treatment of lubricating oil, the process which comprises mixing a lubricating stock with a small percentage of aluminum chloride and with a low boiling halogenated hydrocarbon having not more than a single halogen atom attached to any one carbon atom, subjecting the mixture to a treatment substantially equivalent to that obtained by heating for from 1 to 2 hours at atmospheric pressure and at temperatures 40 ranging from about 150° to 300° F., decanting the resulting sour oil, decomposing traces of aluminum chloride sludge that remain in the sour oil by a method selected from a group consisting of, first, steaming the sour oil with a small amount of clay and with about 0.6 pound of lime per acid number per barrel, second, agitating with sulfuric acid 45 having a concentration of about 5 per cent for a time sufficient to decompose suspended particles of sludge, separating the acid and contacting with clay, third, heating said sour oil to temperatures of about 450° to 550° for a time sufficient to cause suspended sludge to completely react with the oil; then filtering the decomposed particles of sludge 50 from the oil and recovering a finished oil of increased viscosity index, low color N. P. A. and low 55 carbon residue.

3. In the treatment of lubricating oil, the process which comprises mixing a lubricating stock with a small percentage of aluminum chloride and with a low boiling halogenated hydrocarbon having not more than a single halogen atom attached to any one carbon atom, subjecting the mixture to a treatment substantially equivalent to that obtained by heating for from 1 to 2 hours at atmospheric pressure and at temperatures 60 ranging from about 150° to 300° F., decanting the resulting sour oil, decomposing traces of aluminum chloride sludge that remain in the sour oil by a method selected from a group consisting of, first, steaming the sour oil with a small amount of clay and with about 0.6 pound of lime per acid number per barrel, second, agitating with sulfuric acid 65 having a concentration of about 5 per cent for a time sufficient to decompose suspended particles of sludge, separating the acid and contacting with clay, third, heating said sour oil to temperatures of about 450° to 550° for a time sufficient to cause suspended sludge to completely react with the oil; then filtering the decomposed particles of sludge 70 from the oil and recovering a finished oil of increased viscosity index, low color N. P. A. and low 75 carbon residue.

creased viscosity index, low color N. P. A. and low carbon residue.

3. The process of claim 1 wherein the aluminum chloride is added in an amount equal to from 1 to 10 per cent by weight of the lubricating stock.

4. The process of claim 1 wherein the chlorinated hydrocarbon is added in proportions equaling from 5 to 100 per cent by weight of the lubricating stock.

10 5. The process of claim 1 wherein the reaction products obtained are fractionated to remove a portion having low values of gravity and viscosity index.

15 6. In the treatment of lubricating oil, the process which comprises mixing a lubricating stock with a small percentage of aluminum chloride and with a low boiling, halogenated hydrocarbon having not more than a single halogen atom attached to any one carbon atom, subjecting the mixture to a treatment substantially equivalent to that obtained by heating for from 1 to 2 hours at atmospheric pressure and at temperatures ranging from about 150° to 300° F., separating the bulk of the aluminum chloride 20 sludge from the resulting sour oil, steaming the sour oil with a small amount of clay and with about 0.6 pound of lime per acid number per barrel, and filtering.

25 7. In the treatment of lubricating oil, the process which comprises mixing a lubricating stock with a small percentage of aluminum chloride and with a low boiling halogenated hydrocarbon having not more than a single halogen atom attached to any one carbon atom, subjecting the mixture to a treatment substantially equivalent to that obtained by heating for from 1 to 2 hours at atmospheric pressure and at temperatures ranging from about 150° to 300° F., separating the bulk of the aluminum chloride sludge 30 from the resulting sour oil, steaming the sour oil with a small amount of clay and with about 0.6 pound of lime per acid number per barrel, and filtering.

from the resulting sour oil, agitating with dilute sulfuric acid for a time sufficient to decompose suspended particles of sludge; separating the acid, contacting with clay and filtering.

35 8. In the treatment of lubricating oil, the process which comprises mixing a lubricating stock with a small percentage of aluminum chloride and with a low boiling, halogenated hydrocarbon having not more than a single halogen atom attached to any one carbon atom, subjecting the mixture to a treatment substantially equivalent to that obtained by heating for from 1 to 2 hours at atmospheric pressure and at temperatures ranging from about 150° to 300° F., separating the bulk of the aluminum chloride 15 sludge from the resulting sour oil, heating said sour oil to temperatures at which the traces of suspended sludge will completely react with the oil and filtering.

20 9. The process of claim 6 wherein the aluminum chloride is added in an amount equal to from about 1 to 10 per cent by weight of the lubricating stock and the chlorinated hydrocarbon is employed in quantities ranging from about 5 to 100 per cent by weight of said lubricating stock. 25

10 10. The process of claim 8 wherein the aluminum chloride is added in an amount equal to from about 1 to 10 per cent by weight of the lubricating stock and the chlorinated hydrocarbon is employed in quantities ranging from about 5 30 to 100 per cent by weight of said lubricating stock.

11. The process of claim 6 wherein the chlorinated hydrocarbon is selected from a group consisting of amyl chloride and amylene dichlorides. 35

12. The process of claim 8 wherein the chlorinated hydrocarbon is selected from a group consisting of amyl chloride and amylene dichlorides.

EUGENE AYRES.  
HERSCHEL G. SMITH.